# EUROPEAN PATENT SPECIFICATION

(11) **EP 0 935 692 B1**
(45) Date of publication and mention of the grant of the patent: **27.11.2002**
(21) Application number: 97900194.8
(22) Date of filing: 08.01.1997
(51) Int. Cl.: D06M 16/00, D06P 5/02, C11D 3/386, D06L 3/02

(54) **FABRIC TREATED WITH CELLULASE AND OXIDOREDUCTASE**
GEWEBE BEHANDELT MIT CELLULASE UND OXIDOREDUCTASE
TISSU TRAITE AVEC DE LA CELLULASE ET DE L'OXYDOREDUCTASE

(30) Priority: 12.01.1996 DK 2496
(43) Date of publication of application: 18.08.1999
(73) Proprietor: Novozymes A/S, 2880 Bagsvaerd (DK)
(72) Inventor: VOLLMOND, Thomas, DK-2880 Bagsvaerd (DK)
(86) International application number: DK9700002
(87) International publication number: WO97025468

(56) References cited:
- WO-A-94/12619

## Description

The present invention relates to the use of cellulase, in combination with a phenol oxidising enzyme system and certain enhancing agents, for providing a worn look in dyed fabric, especially cellulosic fabric such as denim.

### BACKGROUND ART

The past several years have seen the emergence of a new industry, the so called "jeans stonewashing" segment, generated by the fashion demands of a generation desirous of stylish, but informal and comfortable clothing.

Originally, all of the indigo jeans on the market were stiff and uncomfortable when first purchased, due to the finishing system used for denim fabrics.

The first step in the processing evolution was to sell jeans that had been laundered by the manufacturer. These "pre-washed" jeans had a slightly faded appearance and a softer hand that felt comfortable, as though they had been laundered several times. This trend became fashionable as well, and consumers were willing to pay the extra cost involved for this additional processing.

Not long after the introduction of pre-washed jeans, the idea of using abrasive stones to accelerate the aging process was developed, and "stone washing" became the second step in the evolution. Volcanic stones were included in the wash, or tumbled with the damp garments to wear down the stiffest portions such as belt areas, cuffs, and pockets.

However, the use of stones to abrade jeans is very destructive to equipment and fabric, so today the stones are often substituted with a cellulase treatment, or a combination of stones and cellulase is used to achieve the abraded (worn) look; for reference see "AATCC: Garment Wet Processing Technical Manual", 1994, published by American Association of Textile Chemists and Colorists, pp. 19-21.

The fabric looses strength by using the stone-process described above, and the stone-free cellulase treatment does not alone give the desired worn look, so there is a need in industry for a more gentle process.

### SUMMARY OF THE INVENTION

Surprisingly it has been found that by combining the cellulase treatment with a treatment with a phenol oxidizing enzyme system and an enhancing agent it is possible to achieve the desired worn look in fabric with a minimal strength loss; accordingly the present invention relates to the use of
(a) a cellulase in a concentration corresponding to 0.1-250 µg of enzyme protein per g of fabric; and
(b) simultaneously or subsequently a phenol oxidizing enzyme system and an enhancing agent for providing an abraded look with a reduced strength loss in dyed fabric, in an aqueous medium, wherein the enhancing agent can be described by formula I: or by formula II:
wherein R²⁰-R²², X and R¹-R⁹ are groups as defined in claim 1.

### DETAILED DESCRIPTION OF THE INVENTION

### Bleached versus worn look

Persons skilled in the art of evaluating denim finishing processes, are capable of differentiating between a bleached look and a worn (or abraded) look of denim.

The former is a result of removal (bleaching) of dye from the dyed warp yarn. Since the bleaching takes place on the whole surface of every dyed yarn, the result is a general reduction in colour intensity. Thus, the bleached look of a pair of indigo-dyed jeans is characterised by a lighter blue shade than the corresponding reference.

The latter - the worn look - is a result of a treatment of denim with cellulase and/or pumice stone. This process is characterised by an uneven removal of dye from the fabric, hence it results in a high level of contrast between dyed areas and areas from which dye has been removed.

Typically the worn look is obtained by a process involving cellulase and/or pumice stone, whereas the bleached look can be obtained by a process involving non-enzymatic bleaching agents such as hypochlorite or by a process involving oxidoreductase and an enhancing agent.

The present invention relates to providing a worn but not bleached look, comprising a mild treatment with a cellulase and a simultaneous or subsequent mild treatment with an oxidoreductase and an enhancing agent.

### Dyed Fabric

The invention may be applied to any dyed fabric known in the art, in particular to synthetic fabrics such as polyester or to natural fabrics.

The invention is most beneficially applied to cellulose-containing fabrics, such as cotton, viscose, rayon, ramie, linen, Tencel, or mixtures thereof, or mixtures of any of these fibres, or mixtures of any of these fibres together with synthetic fibres. In particular, the fabric is denim.

The fabric may be dyed with vat dyes such as indigo, or indigo-related dyes such as thioindigo. The fabric may also be dyed with more than one dye, e.g., first with a sulphur dye and then with an indigo dye, or vice versa.

In a most preferred embodiment of the invention, the fabric is an indigo-dyed denim with a sulphur-bottom,(i.e. the denim is first dyed with a sulphur dye and then with an indigo dye); including clothing items manufactured therefrom.

### Cellulases

In the present context, the term "cellulase" refers to an enzyme which catalyses the degradation of cellulose to glucose, cellobiose, triose and other cello-oligosaccharides.

In the present context the term "cellulase" is understood to include a mature protein or a precursor form thereof or a functional fragment thereof which essentially has the activity of the full-length enzyme. Furthermore, the term "cellulase" is intended to include homologues or analogues of said enzyme. Such homologues comprise an amino acid sequence exhibiting a degree of identity of at least 60% with the amino acid sequence of the parent enzyme, i.e. the parent cellulase. The degree of identity may be determined by conventional methods, see for instance, Altshul et al., Bull. Math. Bio. 48, 1986, pp. 603-616, and Henikoff and Henikoff, Proc. Natl. Acad. Sci. USA 89, 1992, pp. 10915-10919.

Preferably, the cellulase to be used in the present invention is a monocomponent (recombinant) cellulase, i.e. a cellulase essentially free from other proteins or cellulase proteins. A recombinant cellulase component may be cloned and expressed according to standard techniques conventional to the skilled person.

In a preferred embodiment of the invention, the cellulase to be used in the method is an endoglucanase (EC 3.2.1.4), preferably a monocomponent (recombinant) endoglucanase.

Preferably, the cellulase is a microbial cellulase, more preferably a bacterial or fungal cellulase.

Examples of bacterial cellulases are cellulases derived from or producible by bacteria from the group of genera consisting of Pseudomonas or Bacillus, in particular Bacillus lautus.

The cellulase or endoglucanase may be an acid, a neutral or an alkaline cellulase or endoglucanase, i.e. exhibiting maximum cellulolytic activity in the acid, neutral or alkaline range, respectively.

Accordingly, a useful cellulase is an acid cellulase, preferably a fungal acid cellulase, which is derived from or producible by fungi from the group of genera consisting of Trichoderma, Actinomyces, Myrothecium, Aspergillus, and Botrytis.

A preferred useful acid cellulase is derived from or producible by fungi from the group of species consisting of Trichoderma viride, Trichoderma reesei, Trichoderma longibrachiatum, Myrothecium verrucaria, Aspergillus niger, Aspergillus oryzae, and Botrytis cinerea.

Another useful cellulase or endoglucanase is a neutral or alkaline cellulase, preferably a fungal neutral or alkaline cellulase, which is derived from or producible by fungi from the group of genera consisting of Aspergillus, Penicillium, Myceliophthora, Humicola, Irpex, Fusarium, Stachybotrys, Scopulariopsis, Chaetomium, Mycogone, Verticillium, Myrothecium, Papulospora, Gliocladium, Cephalosporium and Acremonium.

A preferred alkaline cellulase is derived from or producible by fungi from the group of species consisting of Humicola insolens, Fusarium oxysporum, Myceliopthora thermophila, or Cephalosporium sp., preferably from the group of species consisting of Humicola insolens, DSM 1800, Fusarium oxysporum, DSM 2672, Myceliopthora thermophila, CBS 117.65, or Cephalosporium sp., RYM-202.

A preferred example of a native or parent cellulase is an alkaline endoglucanase which is immunologically reactive with an antibody raised against a highly purified ~43kD endoglucanase derived from Humicola insolens, DSM 1800, or which is a derivative of the ~43kD endoglucanase exhibiting cellulase activity.

Other examples of useful cellulases are variants having, as a parent cellulase, a cellulase of fungal origin, e.g. a cellulase derivable from a strain of the fungal genus Humicola, Trichoderma or Fusarium.

According to the invention the concentration of the cellulase enzyme in the aqueous medium may be 0.1-250 µg of enzyme protein per g of fabric, in particular 0.5-50 µg of enzyme protein per g of fabric.

### Determination of cellulase activity (ECU)

In the context of this invention, cellulase activity can be expressed in ECU. Cellulolytic enzymes hydrolyse CMC, thereby increasing the viscosity of the incubation mixture. The resulting reduction in viscosity may be determined by a vibration viscosimeter (e.g. MIVI 3000 from Sofraser, France).

Determination of the cellulolytic activity, measured in terms of ECU, may be determined according to the following analysis method (assay): The ECU assay quantifies the amount of catalytic activity present in the sample by measuring the ability of the sample to reduce the viscosity of a solution of carboxy-methylcellulose (CMC). The assay is carried out at 40°C; pH 7.5; 0.1M phosphate buffer; time 30 min; using a relative enzyme standard for reducing the viscosity of the CMC (carboxymethylcellulose Hercules 7 LFD) substrate; enzyme concentration approx. 0.15 ECU/ml. The arch standard is defined to 8200 ECU/g.

### Phenol Oxidizing Enzyme Systems

By the term "a phenol oxidizing enzyme system" is meant a system in which an enzyme, by using hydrogen peroxide or molecular oxygen, is capable of oxidizing organic compounds containing phenolic groups. Examples of such enzymes are peroxidases and oxidases.

If the phenol oxidizing enzyme system requires a source of hydrogen peroxide, the source may be hydrogen peroxide or a hydrogen peroxide precursor for in situ production of hydrogen peroxide, e.g., percarbonate or perborate, or a hydrogen peroxide generating enzyme system, e.g., an oxidase and a substrate for the oxidase, or an amino acid oxidase and a suitable amino acid, or a peroxycarboxylic acid or a salt thereof. Hydrogen peroxide may be added at the beginning of or during the process, e.g., in a concentration corresponding to 0.001-25 mM H₂O₂.

If the phenol oxidizing enzyme system requires molecular oxygen, molecular oxygen from the atmosphere will usually be present in sufficient quantity.

The enzyme of the phenol oxidizing enzyme system may be an enzyme exhibiting peroxidase activity or a laccase or a laccase related enzyme as described below.

According to the invention the concentration of the phenol oxidizing enzyme in the aqueous medium may be 0.01-250 µg of enzyme protein per g of fabric, preferably 0.1-250 µg of enzyme protein per g of fabric, in particular 0.5-50 µg of enzyme protein per g of fabric.

### Peroxidases and Peroxidase Acting Compounds

An enzyme exhibiting peroxidase activity may be any peroxidase enzyme comprised by the enzyme classification (EC 1.11.1.7), or any fragment derived therefrom, exhibiting peroxidase activity, or synthetic or semisynthetic derivatives thereof (e.g. porphyrin ring systems or microperoxidases, cf. e.g. US 4,077,768, EP 537 381, WO 91/05858 and WO 92/16634). Such enzymes are known from microbial, plant and animal origins.

Preferably, the peroxidase employed in the method of the invention is producible by plants (e.g. horseradish or soybean peroxidase) or microorganisms such as fungi or bacteria. Some preferred fungi include strains belonging to the subdivision Deuteromycotina, class Hyphomycetes, e.g., Fusarium, Humicola, Tricoderma, Myrothecium, Verticillum, Arthromyces, Caldariomyces, Ulocladium, Embellisia, Cladosporium or Dreschlera, in particular Fusarium oxysporum (DSM 2672), Humicola insolens, Trichoderma resii, Myrothecium verrucana (IFO 6113), Verticillum alboatrum, Verticillum dahlie, Arthromyces ramosus (FERM P-7754), Caldariomyces fumago, Ulocladium chartarum, Embellisia alli or Dreschlera halodes.

Other preferred fungi include strains belonging to the subdivision Basidiomycotina, class Basidiomycetes, e.g. Coprinus, Phanerochaete, Coriolus or Trametes, in particular Coprinus cinereus f. microsporus (IFO 8371), Coprinus macrorhizus, Phanerochaete chrysosporium (e.g. NA-12) or Trametes (previously called Polyporus), e.g. T. versicolor (e.g. PR4 28-A).

Further preferred fungi include strains belonging to the subdivision Zygomycotina, class Mycoraceae, e.g. Rhizopus or Mucor, in particular Mucor hiemalis.

Some preferred bacteria include strains of the order Actinomycetales, e.g., Streptomyces spheroides (ATTC 23965), Streptomyces thermoviolaceus (IFO 12382) or Streptoverticillum verticillium ssp. verticillium.

Other preferred bacteria include Bacillus pumilus (ATCC 12905), Bacillus stearothermophilus, Rhodobacter sphaeroides, Rhodomonas palustri, Streptococcus lactis, Pseudomonas purrocinia (ATCC 15958) or Pseudomonas fluorescens (NRRL B-11) .

Further preferred bacteria include strains belonging to Myxococcus, e.g., M. virescens.

The peroxidase may furthermore be one which is producible by a method comprising cultivating a host cell transformed with a recombinant DNA vector which carries a DNA sequence encoding said peroxidase as well as DNA sequences encoding functions permitting the expression of the DNA sequence encoding the peroxidase, in a culture medium under conditions permitting the expression of the peroxidase and recovering the peroxidase from the culture.

Particularly, a recombinantly produced peroxidase is a peroxidase derived from a Coprinus sp., in particular C. macrorhizus or C. cinereus according to WO 92/16634, or a variant thereof, e.g., a variant as described in WO 94/12621.

In the context of this invention, peroxidase acting compounds comprise peroxidase active fragments derived from cytochromes, haemoglobin or peroxidase enzymes, and synthetic or semisynthetic derivatives thereof, e.g. iron porphins, iron porphyrins, and iron phthalocyanine and derivatives thereof.

### Determination of Peroxidase Activity

1 peroxidase unit (PODU) is the amount of enzyme that catalyzes the conversion of 1 µmole hydrogen peroxide per minute at the following analytical conditions: 0.88 mM hydrogen peroxide, 1.67 mM 2,2'-azinobis(3-ethylbenzothiazoline-6-sulfonate), 0.1 M phosphate buffer, pH 7.0, incubated at 30°C, photometrically followed at 418 nm.

### Laccase and Laccase Related Enzymes

In the context of this invention, laccases and laccase related enzymes contemplate any laccase enzyme comprised by the enzyme classification (EC 1.10.3.2), any chatechol oxidase enzyme comprised by the enzyme classification (EC 1.10.3.1), any bilirubin oxidase enzyme comprised by the enzyme classification (EC 1.3.3.5) or any monophenol mono-oxygenase enzyme comprised by the enzyme classification (EC 1.14.99.1).

The laccase enzymes are known from microbial and plant origin. The microbial laccase enzyme may be derived from bacteria or fungi (including filamentous fungi and yeasts) and suitable examples include a laccase derivable from a strain of Aspergillus, Neurospora, e.g., N. crassa, Podospora, Botrytis, Collybia, Fomes, Lentinus, Pleurotus, Trametes, e.g., T. villosa and T. versicolor, Rhizoctonia, e.g., R. solani, Coprinus, e.g. C. plicatilis and C. cinereus, Psatyrella, Myceliophthora, e.g. M. thermophila, Schytalidium, Polyporus, e.g., P. pinsitus, Phlebia, e.g., P. radita (WO 92/01046), or Coriolus, e.g., C. hirsutus (JP 2-238885).

The laccase or the laccase related enzyme may furthermore be one which is producible by a method comprising cultivating a host cell transformed with a recombinant DNA vector which carries a DNA sequence encoding said laccase as well as DNA sequences encoding functions permitting the expression of the DNA sequence encoding the laccase, in a culture medium under conditions permitting the expression of the laccase enzyme, and recovering the laccase from the culture.

### Determination of Laccase Activity (LACU)

Laccase activity is determined from the oxidation of syringaldazin under aerobic conditions. The violet colour produced is photometered at 530 nm. The analytical conditions are 19 µM syringaldazin, 23.2 mM acetate buffer, pH 5.5, 30°C, 1 min. reaction time.

1 laccase unit (LACU) is the amount of enzyme that catalyses the conversion of 1.0 µmole syringaldazin per minute at these conditions.

### Enhancing Agents

According to the present invention certain enhancing agents are used that enhance the bleaching process. The enhancing agent is an organic compound as defined by the formulas I and II in claim 1.

In particular embodiments, the enhancing agent of formula I is acetosyringone, syringaldehyde, syringic acid, methylsyringate, ethylsyringate, propylsyringate, butylsyringate, hexylsyringate, or octylsyringate.

The enhancing agents described above may be prepared using methods well known to those skilled in the art; some of the enhancing agents are also commercially available, e.g., acetosyringone. Methylsyringate, ethylsyringate, propylsyringate, butylsyringate, hexylsyringate and octylsyringate may be produced as disclosed in Chem. Ber. 67, 1934, p. 67.

The enhancing agent of formula II may be in particular 10-methylphenothiazine, phenothiazine-10-propionic acid, N-hydroxysuccinimide phenothiazine-10-propionate, 10-ethylphenothiazine-4-carboxylic acid, 10-ethylphenothiazine, 10-propylphenothiazine, 10-isopropylphenothiazine, methyl phenothiazine-10-propionate, 10-phenylphenothiazine, 10-allylphenothiazine, 10-(3-(4-methylpiperazin-1-yl)propyl)phenothiazine, 10-(2-pyrrolidin-1-yl-ethyl)phenothiazine, 2-methoxy-10-methyl-phenothiazine, 1-methoxy-10-methylphenothiazine, 3-methoxy-10-methylphenothiazine, 3,10-dimethylphenothiazine, 3,7,10-trimethylphenothiazine, 10-(2-hydroxyethyl)phenothiazine, 10-(3-hydroxypropyl)phenothiazine, 3- (2-hydroxyethyl)-10-methylphenothiazine, 3-hydroxymethyl-10-methylphenothiazine, 3,7-dibromophenothiazine-10-propionic acid, phenothiazine-10-propionamide, chlorpromazine, 2-chloro-10-methylphenothiazine, 2-acetyl-10-methylphenothiazine, 10-methylphenoxazine, 10-ethylphenoxazine, phenoxazine-10-propionic acid, 10-(2-hydroxyethyl)phenoxazine phenoxazine-10-hydroxyethyl, promazine hydrochloride, phenothiazine-10-ethyl-4-carboxy, phenothiazine-10-ethylalcohol or 4-carboxyphenoxazine-10-propionic acid.

The enhancing agents may be obtained from Sigma-Aldrich, Janssen Chimica, Kodak, Tokyo Kasai Organic Chemicals, Daiichi Pure Chemicals Co. or Boehringer Mannheim; N-methylated derivatives of phenothiazine and phenoxazine may be prepared by methylation with methyliodide as described by Cornel Bodea and Ioan Silberg in "Recent Advances in the Chemistry of Phenothiazines" (Advances in heterocyclic chemistry, 1968, Vol. 9, pp. 321-460); B. Cardillo & G. Casnati in Tetrahedron, 1967, Vol. 23, p. 3771. Phenothiazine and phenoxazine propionic acids may be prepared as described in J. Org. Chem. 15, 1950, pp. 1125-1130. Hydroxyethyl and hydroxypropyl derivatives of phenothiazine and phenoxazine may be prepared as described by G. Cauquil in Bulletin de la Society Chemique de France, 1960, p.1049.

The enhancing agent used according to the invention may be present in concentrations of from 0.05 to 500 µmole per g denim, preferably 0.05 to 100 µmole per g denim, in particular 0.05 to 20 µmole per g denim.

### Industrial Applications

The present invention is typically used in industrial machines for cellulase treatment of fabric.

The fabric is normally added to the machine according to the machine capacity per the manufacturer's instructions. The fabric may be added to the machine prior to introducing water or the fabric may be added after water is introduced.

Normally, the cellulase treatment will be performed first, followed by the treatment with the phenol oxidizing enzyme system and the enhancing agent, but the two processes may also be performed simultaneously.

The cellulase may be present in the water prior to adding the fabric or it may be added after the fabric has been wetted. Normally a buffer will be used in order to be close to the pH optimum of the enzyme in question. After the fabric has been contacted with the cellulase it should be agitated in the machine for a sufficient period of time to ensure that the fabric is fully wetted and to ensure the action of the enzyme. Typically a reaction time between 5 and 60 minutes and a reaction temperature between 20°C and 90°C, preferably between 30°C and 80°C, more preferably between 40°C and 70°C, will be suitable.

The phenol oxidizing enzyme system and the enhancing agent of the invention may be present in the water prior to adding the fabric or they may be added after the fabric has been wetted. The phenol oxidizing enzyme system may be added simultaneously with the enhancing agent or they may be added separately. Normally a buffer will be used in order to be close to the pH optimum of the enzyme in question. After the fabric has been contacted with the phenol oxidizing enzyme system and the enhancing agent of the invention it should be agitated in the machine for a sufficient period of time to ensure that the fabric is fully wetted and to ensure the action of the enzyme system and the enhancing agent. Typically a reaction time between 5 and 60 minutes and a reaction temperature between 20°C and 90°C, preferably between 30°C and 80°C, more preferably between 40°C and 70°C, will be suitable.

The above described process steps may be performed once or it may be repeated two or three times depending on how worn the dyed fabric should look.

The invention is further illustrated in the following examples which are not intended to be in any way limiting to the scope of the invention as claimed.

### EXAMPLE 1

### Treatment of denim with cellulase and laccase/enhancing agent:

Treatment of denim was carried out in industrial scale equipment (450 litres) using 50 kg of denim.

5 different types of denim (all manufactured by Levi Strauss & Co) were applied. The 5 types of denim were all of the "sulphur-bottom" type but the ratio between indigo and sulphur dye varied, as did the fabric construction.

### Step 1: Abrasion with cellulase/pumice stone.

The denim was split into 2 different abrasion processes:
1) a standard abrasion process involving neutral cellulase + pumice stone or
2) an abrasion process with no addition of pumice stone.
   1: 750 g MTF12EB (neutral cellulase, available from T.S. Chemicals, UK)
      64 kg pumice stone
      50 minutes, pH 6.5, 60°C
      per 50 kg of denim
   2: 750 g MTF12EB (neutral cellulase, available from T.S. Chemicals, UK) 50 minutes, pH 6.5, 60°C
      per 50 kg of denim

### Step 2: Treatment with laccase and enhancing agent

The jeans from step 1 (except one of each type, which were kept as reference) were then treated with a laccase and an enhancing agent using following dosages and conditions:
270 g mono-sodium phosphate
68 g di-sodium phosphate
40.5 g PPT (10-propionic acid phenothiazine)
40000 LACU (= 625 mg) Trametes villosa laccase, available from Novo Nordisk A/S 12 minutes, pH 6-6.5, 60°C
   per 50 kg of denim

As a result of the treatments, each type of denim resulted in 4 different looks (+/- pumice stone in cellulase treatment and +/- laccase treatment).
The jeans were then subjected to visual evaluation by 6 experts, skilled in the art of evaluating denim finishing processes. The major conclusions from their evaluation were:
The cellulase process without pumice stone resulted in significantly less abrasion than the corresponding process involving pumice stone.
The process consisting of a cellulase treatment step without pumice stone and a subsequent treatment with laccase and enhancing agent resulted in jeans with a highly worn look without having a bleached look. This was evaluated as extremely interesting as the process provides a look that would otherwise require higher amounts of cellulase and addition of substantial amounts of pumice stone. Furthermore, the process provided a highly worn look, without having the fabric damage that would be the result of a pumice stone or cellulase/pumice stone process for obtaining the same look.

### EXAMPLE 2

### Abrasion enhancement with Myceliophthora thermophila laccase and Methyl syringate as enhancing agent

### Fabric:

Swift denim fabric (type Dakota) was used.

### Abrasion:

A 12 kg Wascator FL 120 wash extractor was used for abrasion of the denim.

| | |
|---|---|
| Denim load | 2.6 kg |
| Water | 40 l |
| Buffer | 30 g KH₂PO₄ |
| | 10 g Na₂HPO₄ |
| pH | 6.8 |
| Enzyme | 70 g Denimax™ T (a commercial product, available from Novo Nordisk A/S, Bagsvaerd, Denmark) |
| Time | 2 hours |
| Temperature | 55°C |

### Abrasion enhancement:

A Wascator FOM 71 wash extractor was used for abrasion enhancement of the denim.

| | |
|---|---|
| Denim load | 0.8 kg |
| Water | 20 l |
| Buffer | 4.2 g Sodium acetate, 3 H₂O |
| | 4.0 g Succinic acid |
| pH | 5.1 |
| Enzyme | 670 LACU Myceliophthora thermophila laccase (available from Novo Nordisk A/S) |
| Enhancing agent | 0.5 g Methyl syringate |
| Time | 20 minutes |
| Temperature | 60°C |

### Evaluation:

The results were evaluated visually in a lightbox as well as by measuring the reflection. For the latter a Texflash 2000 (available from Datacolor) was used to evaluate the degree of bleaching and brightening using the change in the color space coordinates L*a*b*:
L gives the change in black (-L*)/white (+L*), a gives the change in green (-a*)/red (+a*), and b gives the change in blue (-b*)/yellow (+b*).

A decrease in L* means an increase in blackness (decrease of white colour), an increase in L* means an increase in whiteness (a decrease in black colour), a decrease in a* means an increase in green colour (decrease in red colour), an increase in a* means an increase in red colour (a decrease in green colour), a decrease in b* means an increase in blue colour (a decrease in yellow colour), and an increase in b* means an increase in yellow colour (a decrease in blue colour).

The Texflash 2000 was operated in the L*a*b* coordinate system. The light source used was a CIE light standard C. Each measurement was an average of 10 measurements. The instrument was calibrated using calibration plates (black and white).

### Results:

The results are shown in the following table (Table 1):

**Table 1**

| Process step | L* | a* | b* | ΔL* |
|---|---|---|---|---|
| Abraded | 31.60 | -1.45 | -17.41 | |
| Abraded and enhanced | 34.88 | -1.69 | -16.64 | 3.28 |

From visual evaluation the abrasion enhancement process produced denim with a highly worn look without having a bleached look, similar to the results obtained in Example 1. Thus, the Mvceliophthora thermophila laccase and the methyl syringate enhancing agent work in a similar manner as the laccase and enhancing agent used in Example 1.

### EXAMPLE 3

### Abrasion enhancement with varying levels of cellulase abrasion and varying dosages of laccase and enhancing agent

### Fabric:

Swift denim fabric (type Dakota) was used.

### Abrasion:

A 12 kg Wascator FL 120 wash extractor was used for abrasion of the denim. 3 different dosages of cellulase were used applied.

| | |
|---|---|
| Denim load | 2.6 kg |
| Water | 40 l |
| Buffer | 30 g KH₂PO₄ |
| | 10 g Na₂HPO₄ |
| pH | 6.8 |
| Enzyme | Denimax™ Ultra MG (a commercial mono-component cellulase product, available from Novo Nordisk A/S) |
| 1 | 8 g (= 3.7 µg cellulase/g fabric) |
| 2 | 28 g (= 12.9 µg cellulase/g fabric) |
| 3 | 54 g (= 24.9 µg cellulase/g fabric) |
| Time | 2 hours |
| Temperature | 55°C |

### Abrasion enhancement:

A Wascator FOM 71 wash extractor was used for abrasion enhancement of the denim. The dosage of laccase and mediator was varied in 3 trials.

| | |
|---|---|
| Denim load | 0.8 kg |
| Water | 20 l |
| Buffer | 4.2 g sodium acetate, 3 H₂O |
| | 4.0 g succinic acid |
| pH | 5.1 |

| Enzyme Trametes villosa laccase (available from Novo Nordisk A/S) | |
|---|---|
| A | 300 LACU (= 5.9 µg laccase/g fabric) |
| B | 600 LACU (= 11.7 µg laccase/g fabric) |
| C | 900 LACU (= 17.6 µg laccase/g fabric) |

| Enhancing agent 10-propionic acid phenothiazine | |
|---|---|
| A | 0.15 g (= 0.7 µmole/g fabric) |
| B | 0.30 g (= 1.4 µmole/g fabric) |
| C | 0.45 g (= 2.1 µmole/g fabric) |
| Time | 20 minutes |
| Temperature | 60°C |

### Evaluation:

As described in Example 2.

### Results:

The results are shown in the following table (Table 2):

**Table 2**

| Cellulase dosage (g) | Laccase dosage (LACU) | Dosage of enhancing agent (g) | L* | ΔL* | Visual evaluation of effect |
|---|---|---|---|---|---|
| 8 | - | - | 28.69 | - | No worn look |
| 8 | 300 | 0.15 | 32.47 | 3.78 | Abrasion enhancement (Worn look) |
| 8 | 600 | 0.30 | 34.23 | 5.54 | Abrasion enhancement (Worn look) |
| 8 | 900 | 0.45 | 35.93 | 7.24 | Bleaching (Bleached look) |
| 28 | - | - | 31.58 | - | No worn look |
| 28 | 300 | 0.15 | 33.90 | 2.32 | Abrasion enhancement (Worn look) |
| 28 | 600 | 0.30 | 35.74 | 4.16 | Abrasion enhancement (Worn look) |
| 28 | 900 | 0.45 | 38.50 | 6.92 | Bleaching (Bleached look) |
| 54 | - | - | 32.91 | - | No worn look |
| 54 | 300 | 0.15 | 35.32 | 2.41 | Abrasion enhancement (Worn look) |
| 54 | 600 | 0.30 | 37.90 | 4.99 | Bleaching (Bleached look) |
| 54 | 900 | 0.45 | 40.46 | 7.55 | Bleaching (Bleached look) |

As it can be seen, to obtain the desired abrasion enhancement it is preferred to keep the dosage of laccase and the dosage of enhancing agent below a certain limit (otherwise the result will be a bleached appearance). Also, it is seen that this limit depends on the dosage of cellulase in the abrasion step - the higher the cellulase dosage, the lower the limit is, i.e. according to the following approximate rules:
at 4 µg mono-component cellulase/g fabric abrasion enhancement is obtained at
   < 15 µg laccase/g fabric and
   < 2 µmole enhancing agent/g fabric;
at 13 µg mono-component cellulase/g fabric abrasion enhancement is obtained at
   < 12 µg laccase/g fabric and
   < 1.5 µmole enhancing agent/g fabric; and
at 25 µg mono-component cellulase/g fabric abrasion enhancement is obtained at
   < 10 µg laccase/g fabric and
   < 1 µmole enhancing agent/g fabric.

## Claims

1. Use of (a) a cellulase in a concentration corresponding to 0.1-250 µg of enzyme protein per g of fabric and (b) simultaneously or subsequently a phenol oxidizing enzyme system and an enhancing agent for providing an abraded look in dyed fabric, in an aqueous medium, wherein the enhancing agent has either formula I: in which R²⁰ is Y, -CH=CH-Y, or -CH=CH-CH=CH-Y, in which Y is selected from the group consisting of-CO-E, -SO₂-E, -N-RR', and -N⁺-RR'R", in which E is -H, -OH, -R, or -OR, and R and R' and R" may be identical or different and are selected from -H or C₁-C₈ alkyl, which alkyl may be saturated or unsaturated, branched or unbranched; and R²¹ and R²² may be the same or different and are selected from CₘH₂ₘ₊₁; 1 ≤ m ≤ 5; or formula II: in which formula X represents (-O-) or (-S-), and the substituent groups R¹- R⁴ and R⁶-R⁹, which may be identical or different, independently represents any of the following radicals: hydrogen, halogen, hydroxy, formyl, carboxy, and esters and salts hereof, carbamoyl, sulfo, and esters and salts hereof, sulfamoyl, nitro. amino, amino-C₁C₅-alkyl, and R¹-R⁹ represents any of the following phenyl, C₁-C₁₄-alkyl, C₁-C₅-alkoxy, carbonyl-C₁-C₅-alkyl, aryl-C₁-C₅-alkyl; which carbamoyl and sulfamoyl groups may furthermore be unsubstituted or substituted once or twice with a substituent group R¹⁰; and which phenyl may furthermore be unsubstituted or substituted with one or more substituent groups R¹⁰; and which C₁-C₁₄-alkyl, C₁-C₅-alkoxy, carbonyl-C₁-C₅-alkyl, and aryl-C₁-C₅-alkyl groups may be saturated or unsaturated, branched or unbranched, and may furthermore be unsubstituted or substituted with one or more substituent groups R¹⁰;
which substituent group R¹⁰ represents any of the following radicals: halogen, hydroxy, formyl, carboxy and esters and salts hereof, carbamoyl, sulfo and esters and salts hereof, sulfamoyl, nitro, amino, phenyl, amlnoalkyl, piperidino, piperazinyl, pyrrolidino, C₁-C₅-alkyl, C₁-C₅-alkoxy;
or in which general formula two of the substituent groups R¹-R⁹ may together form a group -Z-, in which Z represents any of the following groups: (-CHR¹⁰-N=N-), (-CH=CH-)ₙ, (-CH=N-)ₙ or (-N=CR¹⁰-NR¹¹-), in which groups n represents an integer of from 1 to 3, R¹⁰ is a substituent group as defined above and R¹¹ is defined as R¹⁰.

2. The use according to claim 1, wherein the fabric is dyed with a vat dye.

3. The use according to claim 2, wherein the vat dye is indigo or thioindigo.

4. The use according to any of claims 1-3, wherein the fabric is a cellulosic fabric or a mixture of cellulosic fibres or a mixture of cellulosic fibres and synthetic fibres.

5. The use according to any of claims 1-4, wherein the fabric is denim, preferably denim dyed with indigo or thioindigo.

6. The use according to claim 1, wherein the cellulase is obtainable from Humicola, e.g., Humicola insolens, Fusarium, e.g., Fusarium oxysporum, Myceliophthora, e.g., Myceliophthora thermophila, or Cephalosporium sp.

7. The use according to claim 1, wherein the concentration of the cellulase corresponds to 0.5-50 µg of enzyme protein per g of fabric.

8. The use according to claim 1, wherein the phenol oxidizing enzyme system is a peroxidase and a hydrogen peroxide source.

9. The use according to claim 7, wherein the peroxidase is horseradish peroxidase, soybean peroxidase or a peroxidase enzyme obtainable from Coprinus, e.g., C. cinereus or C. macrorhizus, or from Bacillus, e.g., B. pumilus, or Myxococcus, e.g., M. virescens.

10. The use according to claim 8 or 9, wherein the hydrogen peroxide source is hydrogen peroxide or a hydrogen peroxide precursor, e.g., perborate or percarbonate, or a hydrogen peroxide generating enzyme system, e.g., an oxidase and its substrate, or a peroxycarboxylic acid or a salt thereof.

11. The use according to any of claims 1-10, wherein the aqueous medium contains H₂O₂ or a precursor for H₂O₂ in a concentration corresponding to 0.001-25 mM H₂O₂.

12. The use according to claim 1, wherein the phenol oxidizing enzyme system is a laccase or a laccase related enzyme together with oxygen.

13. The use according to claim 12, wherein the laccase is obtainable from Trametes, e.g., Trametes villosa, Coprinus, e.g., Coprinus cinereus, or Myceliophthora, e.g., Myceliophthora thermophila.

14. The use according to any of claims 1-13, wherein the concentration of the phenol oxidizing enzyme corresponds to 0.01-250 µg of enzyme protein per g of fabric, in particular 0.5-50 µg of enzyme protein per g of fabric.

15. The use according to claim 1, wherein the enhancing agent belongs to the group consisting of acetosyringone, syringaldehyde, methylsyringate and syringic acid.

16. The use according to claim 1, wherein the enhancing agent belongs to the group consisting of 10-methylphenothiazine, phenothiazine-10-propionic acid, phenoxazine-10-propionic acid, phenoxazine-10-hydroxyethyl, phenothiazine-10-ethyt-4-carboxy, promazine hydrochloride and phenothiazine-10-ethylalcohol.

17. The use according to any of claims 1-16, wherein the enhancing agent in the aqueous medium is present in concentrations of from 0.05 to 500 µmole per g denim, preferably 0.05 to 100 µmole per g denim.

## Patentansprüche

1. Verwendung von (a) einer Zellulase in einer Konzentration entsprechend 0,1-250 µg Enzymprotein pro g Gewebe und (b) gleichzeitig oder nachfolgend eines Phenol-oxidierenden Enzymsystems und eines Verstärkungsmittels zur Bereitstellung eines verschlissenen Aussehens in gefärbten Fasern, in einem wässerigen Medium, wobei das Verstärkungsmittel entweder die Formel I hat: worin R²⁰ Y, -CH=CH-Y oder -CH=CH-CH=CH-Y ist, worin Y ausgewählt ist aus der Gruppe bestehend aus -CO-E, -SO₂-E, -N-RR' und -N⁺-RR'R", in der E -H, -OH, -R oder -OR ist und R und R' und R" identisch oder verschieden sein können und ausgewählt sind aus -H oder C₁-C₈alkyl, wobei der Alkylrest gesättigt oder ungesättigt, verzweigt oder unverzweigt sein kann; und R²¹ und R²² gleich oder verschieden sein können und ausgewählt sind aus CₘH₂ₘ₊₁; 1 ≤ m < 5; oder Formel II: wobei X in dieser Formel (-O-) oder (-S-) darstellt und die Substituentengruppen R¹-R⁴ und R⁶-R⁹, welche identisch oder verschieden sein können, unabhängig beliebige der folgenden Radikale darstellen: Wasserstoff, Halogen, Hydroxy, Formyl, Carboxy und Ester und Salze hiervon, Carbalogen, Hydroxy, Formyl, Carboxy und Ester und Salze hiervon, Carbamoyl, Sulfo und Ester und Salze hiervon, Sulfamoyl, Nitro, Amino, Amino-C₁-C₅-alkyl und R¹-R⁹ ein beliebiges der folgenden Phenyle darstellen, C₁-C₁₄-alkyl, C₁-C₅-alkoxy, Carbonyl-C₁-C₅-alkyl, Aryl-C₁-C₅-alkyl; wobei die Carbamoyl- und Sulfarnoylgruppen weiterhin unsubstituiert oder ein- oder zweifach mit einer Substituentengruppe. R¹⁰ substituiert sein können; und wobei das Phenyl weiterhin unsubstituiert oder mit einer oder mehreren Substituentengruppen R¹⁰ substituiert sein kann; und wobei die C₁-C₁₄-alkyl-, C₁-C₅-alkoxy-, Carbonyl-C₁-C₅-alkyl- und Aryl-C₁-C₅alkylgruppen gesättigt oder ungesättigt, verzweigt oder unverzweigt sein können und weiterhin unsubstituiert oder mit einer oder mehreren Substituentengruppen R¹⁰ substituiert sein können;
wobei die Substituentengruppe R¹⁰ beliebige der folgenden Radikale darstellt: Halogen, Hydroxy, Formyl, Carboxy und Ester und Salze hiervon, Carbamoyl, Sulfo und Ester und Salze hiervon, Sulfamoyl, Nitro, Amino, Phenyl, Aminoalkyl, Piperidino, Piperazinyl, Pyrrolidino, C₁-C₅-alkyl, C₁-C₅-alkoxy;
oder wobei in dieser allgemeinen Formel zwei der Substituentengruppen R¹-R⁹ zusammen eine Gruppe -Z- bilden können, wobei Z beliebige der folgenden Gruppen darstellt: (-CHR¹⁰-N=N-), (-CH=CH-)ₙ, (-CH=N-)ₙ oder (-N=CR¹⁰-NR¹¹-), wobei in diesen Gruppen n eine ganze Zahl von 1 bis 3 darstellt, R¹⁰ eine wie oben definierte Substituentengruppe ist und R¹¹ wie R¹⁰ definiert ist.

2. Verwendung nach Anspruch 1, wobei das Gewebe mit einem Küpenfarbstoff gefärbt ist.

3. Verwendung nach Anspruch 2, wobei der Küpenfarbstoff Indigo oder Thioindigo ist.

4. Verwendung nach einem beliebigen der Ansprüche 1-3, wobei das Gewebe eine zellulosisches Gewebe oder ein Gemisch aus zellulosischen Fasern oder ein Gemisch aus zellulosischen Fasern und synthetischen Fasern ist.

5. Verwendung nach einem beliebigen der Ansprüche 1-4, wobei das Gewebe Baumwolldrillich, vorzugsweise Baumwolldrillich gefärbt mit Indigo oder Thioindigo ist.

6. Verwendung nach Anspruch 1, wobei die Zellulase erhältlich ist aus Humicola, z.B. Humicola insolens, Fusarium, z.B. Fusarium oxysporum, Myceliophthora, z.B. Myceliophthora thermophila oder Cephalosporium sp.

7. Verwendung nach Anspruch 1, wobei die Konzentration der Zellulase 0,5-50 µg Enzymprotein pro g Gewebe entspricht.

8. Verwendung nach Anspruch 1, wobei das Phenol-oxidierende Enzymsystem eine Peroxidase und eine Wasserstoffperoxidquelle ist.

9. Verwendung nach Anspruch 7, wobei die Peroxidase Meerrettichperoxidase, Sojabohnenperoxidase oder ein Peroxidaseenzym erhältlich aus Coprinus, z.B. C. cinereus oder C. Macrorhizus, oder aus Bacillus, z.B. B. pumilus, oder Myxococcus, z.B. M. virescens, ist.

10. Verwendung nach Anspruch 8 oder 9, wobei die Wasserstoffperoxidquelle Wasserstoffperoxid oder ein Wasserstoffperoxidvorläufer ist, z.B. Perborat oder Percarbonat, oder ein Wasserstoffperoxid-generierendesEnzymsystem, z.B. eine Oxidase und ihr Substrat, oder eine Peroxycarbonsäure oder ein Salz davon.

11. Verwendung nach einem beliebigen der Ansprüche 1-10, wobei das wässerige Medium H₂O₂ oder einen Vorläufer von H₂O₂ in einer Konzentration entsprechend 0,001-25 mM H₂O₂ enthält.

12. Verwendung nach Anspruch 1, wobei das Phenol-oxidierende Enzymsystem eine Laccase oder ein Laccase-verwandtes Enzym zusammen mit Sauerstoff ist.

13. Verwendung nach Anspruch 12, wobei die Laccase erhältlich ist aus Trametes, z.B. Trametes villosa, Coprinus, z.B. Coprinus cinereus, oder Myceliophthora, z.B. Myceliophthora thermophila.

14. Verwendung nach einem beliebigen der Ansprüche 1-13, wobei die Konzentration des Phenol-oxidierenden Enzyms 0,01-250 µg Enzymprotein pro g Gewebe entspricht, insbesondere 0,5-50 µg Enzymprotein pro g Gewebe.

15. Verwendung nach Anspruch 1, wobei das Verstärkungsmittel zu der Gruppe bestehend aus Acetsyringon, Syringaldehyd, Methylsyringat und Syringasäure gehört.

16. Verwendung nach Anspruch 1, wobei das Verstärkungsmittel zu der Gruppe bestehend aus 10-Methylphenothiazin, Phenothiazin-10-propionsäure, Phenoxazin-10-propionsäure, Phenoxazin-10-hydroxyethyl, Phenothiazin-10-ethyl-4-carboxy, Promazinhydrochlorid und Phenothiazin-10-ethylalkohol gehört.

17. Verwendung nach einem beliebigen der Ansprüche 1-16, wobei das Verstärkungsmittel in dem wässerigen Medium in Konzentrationen von 0,05 bis 500 µmol pro g Baumwolldrillich, vorzugsweise 0,05 bis 100 µmol pro g Baumwolldrillich, vorhanden ist.

## Revendications

1. Utilisation (a) d'une cellulose, selon une concentration correspondant à 0,1-250 µg de protéine enzymatique par gramme de tissu, et (b) simultanément, ou ultérieurement, d'un système enzymatique d'oxydation des phénols et d'un agent renforçateur, pour donner un aspect abradé à un tissu teint, dans un milieu aqueux, où l'agent renforçateur a la formule I : dans laquelle R²⁰ est Y, -CH=CH-Y ou -CH=CH-CH=CH-Y, où Y est choisi dans l'ensemble comprenant -CO-E, -SO₂-E, -N-RR' et -N⁺-RR'R" où E est -H, -OH, -R ou -OR, et R et R' et R" peuvent être identiques ou différents et sont choisis chacun parmi -H ou un groupé alkyle en C₁-C₈, lequel groupe alkyle peut être saturé ou insaturé à chaîne droite ou ramifiée ; et R²¹ et R²² peuvent être identiques ou différents et sont choisis chacun parmi CₘH₂ₘ₊₁ ; 1 ≤ m ≤ 5 ;
ou la formule II : dans laquelle formule X représente (-O-) ou (-S-), et les groupes substituants R¹-R⁴ et R⁶-R⁹, qui peuvent être identiques ou différents, représentent chacun indépendamment des autres l'un quelconque des radicaux suivants : hydrogène, halogéno, hydroxy, formyle, carboxy, et leurs esters et sels, carbamoyle, sulfo et leurs esters et sels, sulfamoyle, nitro, amino, amino(alkyle en C₁-C₅), et R¹-R⁹ représentent chacun l'un quelconque des radicaux suivants phényle, alkyle en C₁-C₁₄, alcoxy en C₁-C₅, carbonyl(alkyle en C₁-C₅), aryl (alkyle en C₁-C₅) ; lesquels groupes carbamoyle et sulfamoyle peuvent en outre être non substitués, ou substitués une ou deux fois par un groupe substituant R¹⁰ ; et lequel groupe phényle peut en outre être non substitué, ou substitué par un ou deux groupes substituants R¹⁰ ; et lesquels groupes alkyle en C₁-C₁₄, alcoxy en C₁-C₅, carbonyl (alkyle en C₁-C₅) et aryl (alkyle en C₁-C₅) peuvent être saturés ou insaturés à chaîne droite ou ramifiée et peuvent en outre être non substitués, ou substitués par un ou plusieurs groupes substituants R¹⁰ ;
lequel groupe substituant R¹⁰ représente l'un quelconque des radicaux suivants : halogéno, hydroxy, formyle, carboxy et leurs esters et sels, carbamoyle, sulfo et leurs esters et sels, sulfamoyle, nitro, amino, phényle, aminoalkyle, pipéridino, pipérazinyle, pyrrolidino, alkyle en C₁-C₅, alcoxy en C₁-C₅ ;
ou dans laquelle formule générale deux des substituants R¹-R⁹ peuvent former ensemble un groupe -Z-, où Z représente l'un quelconque des groupes suivants : (-CHR¹⁰-N=N-) , (-CH=CH-)ₙ, (-CH=N-)ₙ ou (-N=CR¹⁰-NR¹¹-), dans lesquels groupes n représente un entier de 1 à 3, R¹⁰ est un groupe substituant tel que défini ci-dessus et R¹¹ est tel que défini pour R¹⁰.

2. Utilisation selon la revendication 1, pour laquelle le tissu est teint avec un colorant de cuve.

3. Utilisation selon la revendication 2, pour laquelle le colorant de cuve est l'indigo ou le thioindigo.

4. Utilisation selon l'une quelconque des revendications 1 à 3, pour laquelle le tissu est un tissu cellulosique ou un mélange de fibres cellulosiques ou un mélange de fibres cellulosiques et de fibres synthétiques.

5. Utilisation selon l'une quelconque des revendications 1 à 4, pour laquelle le tissu est un denim, de préférence un denim teint avec de l'indigo ou du thioindigo.

6. Utilisation selon la revendication 1, pour laquelle la cellulase peut être obtenue à partir de Humicola, par exemple Humicola insolens, Fusarium par exemple Fusarium oxysporum, Myceliophthora, par exemple Myceliophthora thermophila ou Cephalosporium sp.

7. Utilisation selon la revendication 1, pour laquelle la concentration de la cellulase correspond à 0,5-50 µg de protéine enzymatique par g de tissu.

8. Utilisation selon la revendication 1, pour laquelle le système enzymatique d'oxydation des phénols est une peroxydase ou une source de peroxyde d'hydrogène.

9. Utilisation selon la revendication 7, pour laquelle la peroxydase est la peroxydase du raifort, la peroxydase du soja ou une enzyme peroxydase pouvant être obtenue à partir de Coprinus, par exemple C. cinereus ou C. macrorhizus, ou de Bacillus, par exemple B. pumilus, ou Myxococcus, par exemple M. virescens.

10. Utilisation selon la revendication 8 ou 9, pour laquelle la source de peroxyde d'hydrogène est le peroxyde d'hydrogène ou un précurseur de peroxyde d'hydrogène, par exemple un perborate ou un percarbonate, ou un système enzymatique générateur de peroxyde d'hydrogène, par exemple une oxydase et son substrat, ou un acide peroxycarboxylique ou un sel de ce dernier.

11. Utilisation selon l'une quelconque des revendications 1 à 10, pour laquelle le milieu aqueux contient du H₂O₂ ou un précurseur de H₂O₂ à une concentration correspondant à 0,001-25 mM de H₂O₂.

12. Utilisation selon la revendication 1, pour laquelle le système enzymatique d'oxydation des phénols est une laccase ou une enzyme apparentée à la laccase, avec de l'oxygène.

13. Utilisation selon la revendication 12, pour laquelle la laccase peut être obtenue à partir de Trametes, par exemple Trametes villosa, Coprinus, par exemple Coprinus cinereus, ou Myceliophthora, par exemple Myceliophthora thermophila.

14. Utilisation selon l'une quelconque des revendications 1 à 13, pour laquelle la concentration de l'enzyme d'oxydation des phénols correspond à 0,01-250 µg de protéine enzymatique par g de tissu, en particulier 0,5-50 µg de protéine enzymatique par g de tissu.

15. Utilisation selon la revendication 1, pour laquelle l'agent renforçateur appartient à l'ensemble comprenant l'acétosyringone, le syringaldéhyde, le syringate de méthyle et l'acide syringique.

16. Utilisation selon la revendication 1, pour laquelle l'agent renforçateur appartient à l'ensemble comprenant la 10-méthylphénothiazine, l'acide phénothiazine-10-propionique, l'acide phénoxazine-10-propionique, le phénoxazine-10-hydroxyéthyle, le phénothiazine-10-éthyl-4-carboxy, le chlorhydrate de promazine et l'alcool phénothiazine-10-éthylique.

17. Utilisation selon l'une quelconque des revendications 1 à 16, pour laquelle l'agent renforçateur dans le milieu aqueux est présent à des concentrations de 0,05 à 500 µmoles par g de denim, de préférence de 0,05 à 100 µmoles par g de denim.
